# EUROPEAN PATENT APPLICATION

(11) **EP 2 351 865 A1**
(43) Date of publication of application: **03.08.2011**
(21) Application number: 11003390.9
(22) Date of filing: 27.10.2004
(51) Int. Cl.: C22C 37/06, C22C 37/08, C22C 37/10, C22C 33/08

(54) **Improved wear resitant alloy**

(62) Divisional of application: 04789619.6
(71) Applicant: Global Tough Alloys Pty Ltd, Belair, S.A. 5052 (AU)
(72) Inventor: Powell, Graham Leonard Fraser, Belair South Australia 5052 (AU)
(74) Representative: Schicker, Silvia

(57) **Abstract**

A wear resistant, high chromium white iron, in an unheat-treated condition has a microstructure substantially comprising austenite and M7C3 carbides. The white iron contains at least one martensite promoter and at least one austenite stabiliser which are present at respective levels to achieve a balance between their effects whereby the white iron is substantially crack-free. The white iron may be as-cast or comprise well deposited hardfacing.

## Description

### Field of the Invention

The present invention relates to wear resistant, high chromium white irons which are suitable for hardfacing of components and also for direct casting of complete products, and which enable improved fracture toughness.

### Background of the Invention

Chromium white irons, in particular high chromium white irons, resist wear as a result of their content of very hard M₇C₃ carbides, where M is Fe,Cr or Cr,Fe but may include small amounts of other elements such as Mn or Ni, depending upon the composition. The wear resistant high chromium white irons may be hypoeutectic, eutectic or hypereutectic.

The hypoeutectic chromium white irons have up to about 3.0% carbon, and their microstructure contains primary dendrites of austenite in a matrix of a eutectic mixture of M₇C₃ carbides and austenite. The eutectic white irons have from about 3.0% to about 4.0% carbon and a microstructure of a eutectic mixture of M₇C₃ carbides and austenite. The hypereutectic chromium white irons have from about 3.5% to about 5.0% carbon, while their microstructure contains primary M₇C₃ carbides in a matrix of a eutectic mixture of M₇C₃ carbides and austenite. In each case, it is the presence of the M₇C₃ carbides, either as eutectic carbides or primary carbides, that provides the alloy with its wear characteristics. The hypereutectic white irons are considered to have higher volume fractions of the hard and wear resistant M₇C₃ carbides than the hypoeutectic white irons, and are thus often the preferred alloy for many hardfacing applications. However, the hypereutectic white irons generally are not favoured for casting, due to stress induced cracking during cooling.

It is widely recognised in the art that, with the increase in wear resistant properties available with hypereutectic high chromium white irons, there is a corresponding decrease in fracture toughness. High chromium white cast irons are used extensively in mining and mineral processing industries, in applications in which their abrasion resistance is required, but in which relatively low fracture toughness is acceptable. However, there are other applications where low fracture toughness has not been acceptable. This has meant that hypereutectic high chromium white cast irons have not been usable and there have been various attempts to address this.

The background section of Australian patent application AU-A-28865/84, which primarily relates to high chromium white cast irons of both hypoeutectic and hypereutectic compositions, describes the many failed attempts to develop satisfactory hypereutectic white iron alloys for castings, which combine wear resistance with fracture toughness. AU-A-28865/84 also describes various attempts to develop hypoeutectic compositions, and draws on attempts in the art to develop suitable hardfacing alloys as providing possible solutions to the wear resistance vs fracture toughness dilemma. However, AU-A-28865/84 in fact predominantly solves the cracking problem of cast compositions by forming them as cast composites - namely by creating a composite component comprising the preferred alloy metallurgically bonded to a substrate, thus assisting with avoiding the likelihood of cracking upon the cast alloy cooling. Indeed, AU-A-28865/84 seeks to overcome the disadvantages of low fracture toughness and cracking with hypereutectic castings having greater than 4.0 wt.% carbon by ensuring the formation in a composite casting of primary M₇C₃ carbides with mean cross-sectional dimensions no greater than 75 micron, and suggests a variety of mechanisms for doing so. Thus, AU-A-28865/84 aims to overcome the problem by forming composite components and limiting the size of the primary M₇C₃ carbides in the alloy itself.

United States patent 5,803,152 also seeks to refine the microstructure of, in particular, thick section hypereutectic white iron castings, in order to maximise nucleation of primary carbides, thereby enabling an increase not only in fracture toughness but also in wear resistance. This refinement is achieved by introducing a particulate material into a stream of molten metal as the metal is being poured for a casting operation. The particulate material is to extract heat from, and to undercool, the molten metal into the primary phase solidification range between the liquidus and solidus temperatures.

In relation to previous attempts to improve fracture toughness in hardfacing alloys, United States patent 6,375,895 points out that most prior art high chromium white irons for hardfacing always show a more or less dense network of cracks (or check cracking) in the as-welded condition, despite precautions to avoid this. US 6,375,895 indicates that the comparative hardness of primary carbides (about 1700 Brinell hardness number (BHN)) in a soft austenite matrix (about 300 BHN to 600 BHN) gives rise to shrinkage cracks on cooling from the molten state. The solution offered by US 6,375,895 is to adopt a particular alloy composition, pre-heating of the base component to be hardfaced, and subsequent cooling regimes, that ensure a substantial martensitic presence in the microstructure and a consistent hardness (about 455 BHN to 512 BHN) throughout the alloy.

It is an aim of the present invention to provide a wear resistant, high chromium white iron that is able to be cast or used as a hardfacing alloy substantially crack free. When used to produce castings, the white iron of the invention does not require the formation of composite components, or the use of complex casting techniques. Also, the use of costly pre-heating techniques are not necessary for use of the white iron for hardfacing.

Before turning to a summary of the invention, it is to be appreciated that the previous description of prior art is provided only for background purposes. Reference to this prior art is not to be considered as an acknowledgement that the disclosure of any of the documents considered is well known or has entered the realm of common general knowledge in Australia or elsewhere.

### Summary of the Invention

The present inventor has been the first to recognise the causes of the fracture toughness problem with wear-resistant, high chromium white irons. The inventor has recognised the presence of a thin layer of martensite at interfaces between the M₇C₃ carbides and the austenite, and has also recognised that this thin layer of martensite enables or at least initiates cracking. This applies whether the M₇C₃ carbides are primary carbides and the austenite is that of eutectic matrix, or the M₇C₃ carbides are eutectic carbides and the austenite is of the eutectic or, where relevant, the austenite is primary austenite. Thus, the findings apply to hypoeutectic, eutectic and hypereutectic high chromium white irons for use in producing castings. The findings also apply to eutectic and hypereutectic alloys used for weld deposition and for many, if not all, hypoeutectic alloys used for weld deposition.

The inventor has additionally determined that this thin layer of martensite is normally less than 1 micron thick, but may be up to several microns thick, or may be as thin as several nanometres. The layer may not be entirely continuous about a carbide and may not be uniform in thickness. Such a layer will of course only normally be visible using electron microscopes or the like.

Our findings indicate that the presence of the thin layer of martensite ordinarily results in the high chromium white irons from a decrease in chromium and carbon content in the austenite adjacent the M₇C₃ carbides, and the influence of silicon content increasing the tendency for the formation of martensite in the austenite adjacent to the M₇C₃ carbides.

By way of explanation, weld deposits formed during hardfacing are subjected to residual tensile stresses due to shrinkage during cooling after the weld solidifies. We have found that the thin, hard and brittle layer of martensite adjacent the M₇C₃ carbides relieves these tensile stresses by cracking. In the absence of this thin layer of martensite, the softer austenite is able to deform to accommodate the residual tensile stresses, obviating the initiation of cracking and minimising crack propagation where some microcracking still occurs.

The inventor additionally has found that martensite at the interfaces between M₇C₃ carbides and austenite is not the sole cause of cracking of castings and weld deposited hardfacing. A further major cause, as detailed later herein, is the formation of M₇C₃ carbides having a high level of interconnectivity. Some alloy additions are found to increase interconnectivity of the M₇C₃ carbide where the level of at least one of the additions is such that undercooling of the melt occurs before solidification. This applies to both castings and to weld deposits and where this is in conjunction with the presence of martensite at M₇C₃ carbide and austenite interfaces, crack initiation and propagation essentially is unable to be avoided. Where M₇C₃ carbide interconnectivity occurs in alloys which are not prone to the presence of martensite at those interfaces, that source of crack initiation is avoided, although crack initiation and propagation still is largely unavoidable.

The inventor has found that, in large part, the solution to both sources of crack initiation and propagation in high chromium white irons, whether used in castings or weld deposition, is the same.

The present invention provides a wear resistant, high chromium white iron, wherein said white iron in an unheat-treated condition has a microstructure substantially comprising austenite and M₇C₃ carbides and wherein said white iron contains at least one martensite promoter and at least one austenite stabiliser, with said martensite promoter and austenite stabiliser being present at respective levels to achieve a balance between their effects whereby the white iron in an unheat-treated condition has a microstructure characterised by at least one of:
i) being substantially free of martensite at interfaces between the austenite and M₇C₃ carbides; and
ii) having a relatively low level of interconnectivity between carbide particles; such that the white iron is substantially crack-free. In most, if not substantially all instances, the white iron not only is substantially crack-free but also has improved fracture toughness.

In one form, the white iron is in an as-cast condition and said respective levels achieve a balance whereby the white iron is substantially free of martensite at interfaces between the austenite and M₇C₃ carbides.

In another form, the white iron comprises hardfacing provided over a substrate by weld deposition, and the hardfacing is substantially free of check cracking. The balance between the effects of the martensite promoter and the austenite stabiliser may be such that M₇C₃ carbides of said microstructure exhibit a relatively low level of interconnectivity between carbide particles. The low level of interconnectivity preferably is such that the microstructure is substantially free of branched carbide particles and, where relevant, said respective levels also achieve a balance whereby the white iron is substantially free of martensite at interfaces between the austenite and M₇C₃ carbides.

The present invention provides wear-resistant, high chromium white iron alloys having substantially no martensite at interfaces between the M₇C₃ carbides and austenite such that the alloys, either as-cast or as deposited for hardfacing, are substantially crack free. However, it is to be appreciated that reference to there being substantially no martensite at those interfaces does not preclude the presence of some martensite within austenitic regions away from the interfaces. The invention is characterised by the prevention of the formation of the thin layer of martensite at interfaces between the M₇C₃ carbides and austenite, and does not necessitate the total exclusion of all martensite, although this may occur. Indeed, in some compositions the presence of martensite other than at those interfaces is desirable.

In another form, the present invention provides a wear-resistant, high chromium white iron having a sufficient balance of at least one martensite promoter and at least one austenite stabiliser such that there is substantially no martensite at interfaces between the M₇C₃ carbides and austenite such that the white iron, either as-cast or as-deposited for hardfacing, is substantially crack free.

Silicon, as a martensite promoter, is a member of the group of alloying elements that act to promote the formation of martensite. Alloying elements of that group also include boron. In high chromium white irons according to the present invention, silicon is the martensite promoter of principal importance for the purpose of achieving the required balance with the at least one austenite stabiliser. However, boron can be used as a martensite promoter, such as up to about 1% or even as high as 2%. The boron can influence the action of silicon, or it can be used as the sole martensite promoter. In general, the control required by the invention is described herein with reference to silicon as the martensite promoter and to the at least one austenite stabiliser, although it is to be borne in mind that boron can be used as martensite promoter.

The at least one austenite stabiliser is a member of the group of alloying elements that act to promote and stabilise the formation of austenite. Alloying elements of that group include manganese, nickel, copper and molybdenum. These elements can be used alone or in combination. Of these four elements, manganese and nickel are found to be particularly beneficial for the purpose of the present invention. The control required by the invention therefore is described with reference to manganese and/or nickel as the austenite stabiliser, although minor amounts of at least one of the other austenite stabilisers can be present in addition. Also, it is to be borne in mind that the other stabilisers can be used instead of manganese and/or nickel.

In a preferred form of the invention, the thin layer of martensite at interfaces between M₇C₃ carbides and austenite is avoided by a `sufficient balance' of various alloying elements, in the form of suitable amounts of austenite stabilisers (such as manganese and/or nickel) and martensite promoters (such as silicon and/or boron). The term 'sufficient balance' is a functional reference to the amount of those alloying elements that are present in the chromium white iron such that a resultant casting or hard-facing is substantially crack free.

With further regard to these alloying elements, martensite promoters such as silicon have been suggested for addition to some chromium white irons to increase the fluidity of the melt during hardfacing or casting. However, the present inventor has also determined that the presence of a martensite promoter such as silicon can produce a previously unsuspected cumulatively deleterious result. It has been found that the presence of the martensite promoter can have the opposite effect to the preferred austenite stabilisers (manganese and nickel) upon the formation of martensite. Thus, it has been found that the martensite promoter can act not merely to promote the formation of martensite, but specifically to promote martensite formation at interfaces between austenite and M₇C₃ carbides. Hence the reason for the balance of martensite promoter, such as silicon, and austenite stabilisers.

Despite being known to promote martensite, silicon is added or tolerated to substantial levels because its effect as a martensite promotor has been believed to be offset by the use of austenite stabilisers. That is, the perception has been that sufficient austenite stabilisation is able to be achieved, despite the presence of silicon, such that the net result is that the beneficial effect of silicon in increasing melt fluidity is able to be achieved without disadvantage. This perception is supported by the commonly used metallographic techniques. For chromium white irons in which martensite suppression has been sought, the resolution of photomicrographs obtained by those techniques show primary austenite and eutectic matrix for hypoeutectic irons and primary M₇C₃ carbides and eutectic matrix for hypereutectic irons. The resolution is such that, the eutectic is perceived as comprising M₇C₃ carbides and austenite, without martensite. In the case of dendrites of hypoeutectic white irons, those resolutions may show primary dendrites as comprising austenite alone or as comprising austenite within which there may be regions of martensite, as anticipated. In the latter case, the martensitic regions would be considered to be acceptable, given that they are contained within austenite. In each case, the photomicrographs show what is expected and there is no reason to look further as cracking appears to be satisfactorily explained by residual stress.

As indicated, we have found that silicon is able to have an active, if previously unsuspected, role in promoting the formation of martensite despite austenite stabilisation. That role is deleterious in that the martensite formed is at the interfaces between M₇C₃ carbides and austenite. This can be carbides and austenite of the eutectic phase, or primary austenite and eutectic carbide or primary carbide and eutectic austenite, or relevant combinations of these situations.

It remains desirable to have a silicon content which has the known beneficial effect of increasing fluidity. However, it is not simply a matter of having a required level of silicon for this purpose and offsetting the adverse action of silicon as a martensite promoter by adding at least a sufficient excess of austenite stabilizer. One factor is the added cost of excess austenite stabiliser. However a more important reason is provided by a further complex influence of silicon on the microstructure. We have found that, depending on the level at which silicon is present, silicon can either increase or decrease the interconnectivity of M₇C₃ carbides. This is of particular relevance to hypereutectic white irons, but also applies to hypoeutectic irons.

In the section under the heading "High-Chromium White Irons" at page 681, ASM Handbook, Volume 15, Castings, 9th Edition, these white irons are said to be "distinguished by the hard, relatively discontinuous M₇C₃ eutectic carbides". In the case of hypereutectic irons, there also are large hexagonal rods of primary M₇C₃ carbides, and these also are perceived to be at least substantially discontinuous. However, as indicated herein, silicon can influence the extent of carbide interconnectivity, both within eutectic carbide and within primary carbide. An increase in M₇C₃ carbide interconnectivity increases overall brittleness and facilitates crack initiation and propagation, while a decrease in interconnectivity enables the tough austenite phase to limit both crack initiation and propagation.

Silicon can increase the undercooling in the melt before solidification occurs which increases interconnectivity of eutectic M₇C₃ carbides and, for hypereutectic microstructures, increases the interconnectivity of primary M₇C₃ carbides. Overall brittleness of a casting or weld deposit therefore increases. However, if silicon is present at a controlled level such that no substantial undercooling occurs, it has been found that the silicon can serve to decrease the interconnectivity of the primary M₇C₃ carbides and of eutectic M₇C₃ carbides. With such decrease in interconnectivity, fracture toughness, wear resistance and the resistance to thermal shock are increased. Higher levels of silicon can be applied to reduce the interconnectivity of eutectic M₇C₃ carbides in hypoeutectic compositions as the complex regular eutectic with high interconnectivity does not form in hypoeutectic alloys.

We have found that there is a further factor, of particular relevance to casting, which preferably can be taken into account in determining the level of silicon. In current practice, a slow cooling rate is used in casting chromium white irons. In relation to those irons, it is stated at page 683 of the above-detailed ASM Handbook under the heading "Shakeout Practices" that "Cooling all the way to room temperature in the melt is desirable and can be a requirement to avoid cracking, especially if martensite forms during the last stages of cooling". It further is indicated that this precaution can be mandatory in heavy-section castings, and that a frequent cause of high residual stresses and of cracking is extracting castings from the mould at too high a temperature. That is, cracking principally has been attributed to cooling rate, with slower cooling rates reducing the risk of crack formation and propagation.

Our finding is that, subject to the balance between the at least one martensite promoter, such as silicon, and the at least one austenite stabiliser, an increasing level of silicon enables an increasingly higher cooling rate to be used without risk of cracking. This, of course, is of practical benefit in shortening the foundry production cycle time. However, the finding also is of relevance to welding, in which a high cooling rate is inherent, as a higher silicon content for example further diminishes the risk of cracking due to residual stresses without considering the combined effect of silicon level and cooling rate on M₇C₃ interconnectivity.

Taking the above factors into account, it is preferred that the level of silicon in chromium white irons according to the invention is from 0.25 to 3.5%. However, more preferably the level is from 0.5 to 3.25%. In some forms (depending on microstructure), the silicon levels should not be higher than about 2.75%, as will be explained below. Boron is somewhat more potent than silicon and, as indicated above, boron need only be present at levels up to about 1%, or only up to about 2%.

Throughout this specification, unless indicated to the contrary the percentages are by weight. For hard facing applications, the percentages allow for dilution by the base metal, such as from 10 to 40%.

In a particularly preferred form of the invention, the austenite stabilisers manganese and nickel are both present in the alloy in an amount of from 4.0% to about 12%, such as from 4.0% to 8.0% in order to assist in preventing the transformation of austenite to the martensite. However, it is to be understood that it is not essential for both to be present - as the presence of only one of these elements, in the preferred range mentioned, can suffice. Also, while manganese and/or nickel can be present at up to about 12% in at least some instances the preferred range is from 4.0% to 8.0%.

When the alternative austenite stabilisers are used, copper typically can be used at substantially the same levels as indicated for manganese and/or nickel. Molybdenum however needs to be used at higher levels to allow for a proportion which forms carbide and, hence, is not available as austenite stabiliser. Thus, it is appropriate to consider an equivalence of molybdenum which provides similar austenite stabilisation to the other alloy additions. However, it is preferred that the two alternatives, if used at all, be used in combination with manganese and/or nickel, and at a relatively low level. This is particularly so with molybdenum in view of its cost.

It is preferred that, where two or more austenite stabilisers are used in combination, the total level of austenite stabiliser is not in excess of about 20%, and more preferably is not in excess of about 16%.

The balance required by the present invention necessitates control of a number of variables. These include the level of silicon, the level of manganese and the level of nickel. Manganese and nickel can be regarded as the one variable, given that in large part they are interchangeable. However, they do differ slightly in their effectiveness as austenite stabilisers, and it therefore is preferred to regard the levels of manganese and nickel as separate variables. A fourth variable is cooling rate. However, as a variable, cooling rate has greater relevance in casting, as the scope for its variation is somewhat limited in weld deposition.

Current indications are that an empirical relationship between the four variables detailed above may be able to be developed. If so, the form of such relationship is unclear, although it appears clear that none of the currently known or used relationship, such as Andrew's relationship for determining the martensite start temperature Mₛ, is relevant to achieving the balance required by the invention. The end result is that, for a high chromium white iron having a given content of each of carbon and chromium, it is necessary to conduct preliminary routine trial castings and weld depositions to determine a suitable balance between silicon and at least one of manganese and nickel. These trials should be conducted at a cooling rate relevant to a production run for which an overall white iron composition is to be settled. Also, in at least some instances, the silicon content will be predetermined and, subject to this not being at a level likely to result in undercooling, the trials thus may reduce to adjusting the manganese and/or nickel content to achieve the required balance.

As a preliminary measure at least, attainment of the balance can be determined by presenting a magnet to the trial casting or weld deposit. If ferromagnetism (indicative of the presence of martensite in the present context) is not evident, at least approximate attainment of the balance has been achieved. However, it is appropriate to proceed beyond this to a metallographic examination to confirm that there is no martensite at the interface between the M₇C₃ carbides and the austenite.

In the high chromium white iron of the present invention, the amount of chromium present is preferably from 8% to 50%. More preferably the chromium level is from 10% to 30%. The carbon content will typically be from 1.0% to 6.0%. However, there are overlapping sub-ranges for the level of carbon, depending upon whether the white iron is of hypoeutectic, eutectic or hypereutectic composition. The carbides will thus be predominantly of the M₇C₃ type, although small amounts of less hard M₂₃C₆ carbides can be present, such as in primary austenite regions.

For a hypoeutectic chromium white iron composition the amount of carbon present usually will be from 1.0% to 3.0%. For a eutectic composition the amount of carbon present will usually be from 3.0% to 4.0%, while a hypereutectic composition usually will have from 3.5% to 5.0%. However, it will be appreciated that these ranges may alter, depending upon the presence of other alloying elements. For instance, if the alloy includes an amount of up to about 10% (total) niobium and/or vanadium (which might be added to precipitate hard niobium and vanadium carbides to increase wear resistance), then the relevant amounts of carbon present in the respective compositions will shift as follows:

| | |
|---|---|
| Hypoeutectic | 2.0% to 4.0% |
| Eutectic | 4.25% to 4.75% |
| Hypereutectic | 5.0% to 6.0% |

There can be further shifting of these ranges, depending on alloying elements. A person skilled in the art will understand how, and in what circumstances, these ranges will shift. However, some explanation is provided in relation to Figure 1.

### General Description of the Drawings

In order that the invention may more readily be understood, reference now is directed to the accompanying drawings, in which:
Figure 1 shows the liquidus surface projections for chromium white irons in the region of commercial interest;
Figure 2 is a photomicrograph of a sample taken from a hypereutectic casting according to our form of current practice;
Figure 3 is a photomicrograph of part of the field of Figure 2, but at a higher magnification;
Figure 4 is a photomicrograph of a part of the field of Figure 2, but at a still higher magnification;
Figure 5 is a photomicrograph of a sample taken from a hypereutectic casting using a chromium white iron composition according to the present invention;
Figure 6 is a photomicrograph of a sample taken from the same casting as Figure 5, but at a higher magnification;
Figure 7 is a macrograph illustrating check cracking in sample I and typical of weld deposited hardfacing of current practice;
Figures 8(a) and (b) are photomicrographs of the sample shown in Figure 7;
Figure 9 is a photomicrograph of sample II of hardfacing of current practice, showing desirable but non-representative microstructure;
Figure 10 is a photomicrograph of sample III of hardfacing of current practice, showing typical, but undesirable microstructure of that practice;
Figures 11 (a) and 11 (b) are photomicrographs at respective magnifications, showing a check crack through undesirable microstructure of sample II of Figure 9;
Figures 12 and 13 are respective photomicrographs showing undesirable microstructures for sample III of Figure 10;
Figure 14 is an electron micrograph of sample III of Figure 10, showing a typical further undesirable microstructural feature;
Figure 15 is a photomacrograph of a weld deposit typical of a high chromium white iron according to the present invention;
Figure 16 is a photomicrograph taken longitudinally of the direction of application of the weld deposit shown in Figure 15; and
Figure 17 is a photomicrograph taken transversely of the weld deposit shown in Figure 15.

### Detailed Description

Figure 1 illustrates the liquidus surface projections for ternary Fe-Cr-C for high chromium white irons at the Fe-rich corner of metastable C-Cr-Fe liquidus surface. The ternary compositions have up to 6% carbon and up to 40% chromium. They also contain small percentages of manganese and silicon.

The liquidus surface projections in Figure 1 can be used to show the relationship between microstructure and content of carbon and chromium. The region marked y indicates hypoeutectic compositions. The compositions at points A, B, C, D and E all fall within general ranges herein referred to as Group I.

Compositions A and B fall into the hypoeutectic region and are close to the boundaries. Eutectic microstructures fall on the line from U₁ to U₂, from a composition close to B along the line to point C. Hypereutectic compositions are within the region marked M₇C₃, which includes compositions D and E.

Any cooling regime that tends to enhance or promote the transition of austenite to martensite preferably is avoided. For some compositions it may be preferred to adopt a cooling regime that will not promote the formation of martensite. However, as detailed earlier herein, higher silicon contents can enable faster cooling rates.

### Detailed Description of Preferred Embodiments

Illustrative, non-limiting examples of chromium white iron compositions for use in castings or weld deposits in accordance with the present invention are set out in Tables I and II. Table I sets out the compositions of Group I, which cover the compositions at points A, B, C, D and E shown in Figure 1. Table II covers similar compositions that for reasons detailed above, differ in that they include niobium and/or vanadium.

**Table I - Group I Composition Ranges**

| **Microstructure** | **C%** | **Cr%** | **Nb/V %** | **Mn%** | **Ni %** | **Si %** |
|---|---|---|---|---|---|---|
| Hypoeutectic | 1.0 to 3.0 | 18.0 to 27.0 | nil | 4.0 to 8.0 | 4.0 to 8.0 | 0.25 to 2.75 |
| Eutectic | 3.0 to 4.0 | 15.0 to 27.0 | nil | 4.0 to 8.0 | 4.0 to 8.0 | 0.25 to 2.75 |
| Hypereutectic | 4.0 to 5.0 | 20.0 to 27.0 | nil | 4.0 to 8.0 | 4.0 to 8.0 | 0.25 to 3.25 |

**Table II-Group II Composition Ranges**

| **Microstructure** | **C%** | **Cr%** | **NbN %** | **Mn%** | **Ni %** | **Si%** |
|---|---|---|---|---|---|---|
| Hypoeutectic | 2.5 to 4.0 | 18.0 to 27.0 | 10.0 | 4.0 to 8.0 | 4.0 to 8.0 | 0.25 to 2.75 |
| Eutectic | 4.25 to 4.75 | 15.0 to 27.0 | 10.0 | 4.0 to 8.0 | 4.0 to 8.0 | 0.25 to 2.75 |
| Hypereutectic | 5.0 to 6.0 | 20.0 to 27.0 | 10.0 | 4.0 to 8.0 | 4.0 to 8.0 | 0.25 to 3.25 |

| | | | | | | |
|---|---|---|---|---|---|---|
| Notes: 1. In the ranges for each of Tables I and II, the balance of the composition is iron and incidental impurities. However, alloying elements may be added as mentioned above. 2. In the ranges for Table II, niobium and the vanadium may both be provided in amounts within the range of up to 10%, with the preferred total amount being 10%. Also, the carbides resulting from the introduction of the Nb and/or V necessitates the additional carbon shown. | | | | | | |

### Illustrative Examples - Castings

A high chromium white iron casting, which had been subjected to industrial use was cut up to provide segments from which specimens for microstructural characterisation were obtained. The segments were cut using abrasive water-jet cutting. The specimens were cut from the segments with a thin carborundum rotating disc (wafer disc) cooled with copious amounts of a water based coolant. The specimens were examined using an Olympus reflected light microscope at magnifications up to and including X500. The specimens were examined in the unetched and etched conditions. The etchant was acid ferric chloride (5g FeCl₃, 10ml HCl, 100ml H₂O)

Figure 2 is a photomicrograph of polished and acid ferric chloride etched section of a specimen taken from the industry casting. The field of Figure 2 is at the intersection of a subsurface crack and a surface breaking crack. These are large cracks and probably occurred during cooling down after solidification of the casting. A higher resolution photomicrograph of the same section, taken just to the left of the intersection between the cracks, is shown in Figure 3.

The microstructure of Figures 2 and 3 shows the industry casting to be in the as-cast condition. The chromium white iron of the industry casting from which Figures 2 and 3 were derived was a hypereutectic composition shown in Table III.

**Table III**

| Industry Casting Composition % | | | | | | | |
|---|---|---|---|---|---|---|---|
| C | Mn | Si | Ni | Cr | Mo | Cu | Fe/Impurities |
| 4.5 | 1.90 | 0.49 | 0.12 | 34 | 0.95 | 0.07 | Balance |

As can be recognised from Figures 2 and 3, the microstructure exhibits only primary M₇C₃ carbide and austenite at the respective magnifications shown. The microstructure thus is significantly different to that of the usual high chromium white iron despite similar white iron composition. In Figures 2 and 3, there is no regular M₇C₃ eutectic carbide within the austenite. In the case of a regular eutectic, it is the growth of one eutectic phase which enriches the solution to form the second phase. This difference is believed to be due to innoculation of the melt from which the industry casting was made, with the effect of the inoculant being to nucleate M₇C₃ carbide during solidification. The driving force for the growth of the carbide was sufficient for the carbide to solidify independently of the austenite and, hence, a divorced eutectic resulted.

The microstructure shown in Figures 2 and 3 has primary M₇C₃ carbides (white) in a divorced eutectic microstructure. A complex regular structure, with its interconnected carbide rods, has been avoided. This is beneficial since the preferred crack path in high chromium white iron weld deposits and castings is along the interface between the M₇C₃ carbides and the austenite. The interconnected complex regular eutectic carbide structure provides long continuous paths along which cracks can propagate, making elimination of that structure desirable. However, despite this being achieved in the as cast microstructure shown in Figures 2 and 3, cracking still has occurred. The reason for this is evident from Figure 4.

The higher magnification of Figure 4 was taken just above the intersection of the cracks shown in Figure 2, just to the right of the vertical crack. In Figure 4, the lighter coloured phase is the primary M₇C₃ carbide, while the darker matrix predominantly is divorced eutectic austenite. However, the edge regions of the austenite, at interfaces between the austenite and M₇C₃ carbide, have a layer of martensite indicated by black arrows. Also, the white arrow is pointing to a region of precipitated M₂₃C₆ carbide within the austenite.

The martensite forms a continuous layer at the M₇C₃ carbide - austenite interfaces, as has been established by transmission electron microscopy (TEM). In Figure 4, the black arrows only indicate regions where the martensite is resolvable at the magnification of Figure 4. Indeed, TEM shows that the martensite layer is actually composed of two very thin martensite layers. These include a thin, very brittle high carbon martensite layer adjacent to the M₇C₃ carbide and a layer of less brittle, lower carbon martensite adjacent to the austenite. However, even at the resolution of Figure 4, some martensite needles can be seen extending some distance from the interface into the austenite.

To minimise cracking, the composition of most commercial high chromium white iron castings is limited to compositions up to eutectic composition. However it is generally accepted that the wear rate of high chromium white irons is directly related to the volume fraction of M₇C₃ carbide, both primary and eutectic, and therefore hypoeutectic alloys and eutectic alloys have a higher wear rate than hypereutectic alloys in most circumstances. The choice of the hypoeutectic and eutectic compositions can minimise cracking by minimising the interfacial area between the M₇C₃ carbide and the austenite, which we find is the preferred crack path due to the interfacial layer of martensite. The commercial alloy of Figures 2 to 4 has a hypereutectic composition and, as indicated, the sample supplied contained cracks and interfacial martensite.

High chromium white irons according to the present invention can be hypoeutectic, eutectic or hypereutectic, and can be used in either the as-cast or heat-treated condition. Two compositions of hypereutectic have been trialled using small slowly cooled crucible castings. A micrograph of an acid ferric chloride etched sample from one of the small slowly cooled crucible castings is shown in Figure 5, while the trialled compositions are set out in Table IV.

**Table IV**

| Hypereutectic Casting Compositions | | | | | | |
|---|---|---|---|---|---|---|
| According to the Invention | | | | | | |
| | C | Mn | Si | Cr | Ni | Fe/Impurities |
| Alloy 1: | 4.25 | 9.31 | 2.18 | 27.45 | 4.07 | Balance |
| Alloy 2: | 4.73 | 11.16 | 1.39 | 28.56 | 8.46 | balance |

There are important features in Figure 5. The light etched phase is the hexagonal primary M₇C₃ carbide rods and these are surrounded by an austenite halo. At the resolution of Figure 5 (which is similar to that of Figure 2) there does not appear to be a dark layer of interfacial martensite at the interface between either the primary or eutectic M₇C₃ carbides and the austenite. Figure 6 enables closer scrutiny using optical microscopy (at a resolution better than Figure 4), but also failed to reveal any martensite at the interface. The large volume of primary carbides in the microstructure indicates that the alloy is of hypereutectic composition. As stated earlier, the wear resistance increases with increasing volume fraction of carbides, particularly primary carbides.

In spite of the porosity and the hypereutectic composition there were no indications that the crucible castings contained any cracks.

Thus, in summary, the industry casting microstructure of Figures 2 to 4 contained fine primary M₇C₃ carbide in a divorced austenitic matrix indicating it was of hypereutectic composition and in the as-cast condition. The industry casting microstructure had an interfacial layer of martensite between the M₇C₃ carbide and the austenite. Due to the relatively slow cooling rate of the industry casting the martensite layer could be resolved in the optical microscope. The present invention enables the interfacial martensite to be avoided.

In contrast, the microstructure of the slowly cooled castings of the trial compositions according to the present invention showed that the castings were of hypereutectic composition, that the castings did not show any evidence of martensite at the interfacial regions and that there were no cracks evident.

While the compositions in accordance with the invention were not subjected to TEM, a further simple test is able to show the presence or absence, respectively, of martensite in the microstructure of Figures 2 to 4, and that of Figures 5 and 6. With each of the hypereutectic chromium white irons, the only ferromagnetic phase potentially present in the as-cast condition is martensite. The industry casting from which the photomicrographs of Figures 2 to 4 were derived was ferromagnetic and able to strongly attract a magnet, clearly indicating the presence of martensite. The casting from which Figures 5 and 6 were derived and other castings based on the compositions of Table IV did not attract a magnet, clearly indicating the absence of martensite.

### Illustrative Examples - Weld Deposition

With weld disposition or hardfacing, the invention again enables the substantially complete prevention of formation of a martensite layer at the interfaces between M₇C₃ carbides and austenite. This is achieved in essentially the same way as described for castings, by a suitable balance between silicon as a martensite promotor and the austenite stabilisers manganese and nickel. However, in weld deposition, a further significant benefit can be achieved. This is the avoidance of check cracking as a consequence of the prevention of martensite formation and also a reduction in the level of interconnectivity of M₇C₃ carbides. The latter result is illustrated in the following.

Several industry samples consisting of a weld deposited overlay of a hypereutectic high chromium white iron hardfacing, on a steel substrate, were examined. In each case, the white iron hardfacing exhibited check cracking. The macrograph of Figure 7 provides a good representative illustration of the check cracking. As is evident in Figure 7 the check cracking extended over the entire hardfacing, in a 5 to 10mm mesh, as confirmed by the cm rule shown. In most instances, the cracks extended radially through the thickness of the hardfacing to the substrate-hardface interface.

Identical sample preparation techniques were used for each of the industry samples. The preparation of samples involved selecting sections and plasma cutting them to a size suitable for manipulation in an abrasive cutter. Samples for metallographic examination were sectioned using a carborundum abrasive disk and water based lubricant at a suitable distance from the plasma cut region to ensure no microstructural changes took place due to heating during cutting. Approximate 25 millimetres long by 10 millimetres wide sections were taken transversely and longitudinally to the direction of the weld beads. The viewing plane of the transverse samples is across consecutive weld beads and along a weld bead for the longitudinal sample. These sections were polished using five grades of silicon carbide paper and polished to a 1-micron finish using diamond paste. The polished samples were etched in acid ferric chloride (5g FeCl₃, 10ml HCl, 100ml H₂O for viewing under an optical light microscope.

Representative industry samples of the hardfacing shown in Figure 7 were taken transversely and longitudinally to the weld beads and metallographically prepared. Figures 8a and 8b show the respective microstructures in which acid ferric chloride etching shows the hypereutectic composition of the high chromium white iron is indicated by the presence of primary M₇C₃ carbides. The chemical composition of the hardfacing shown in Figure 7 is identified in Table V as Sample I, with the composition of the hardfacing of some other industry samples being shown as samples II and III.

**Table V**

| Industry Hardfacing Compositions | | | | | |
|---|---|---|---|---|---|
| Sample | C | Si | Cr | Mn | Fe/Impurities |
| I | 4.9 | 0.94 | 27.3 | 1.2 | Balance |
| II | 5.0 | 1.1 | 25.2 | 1.34 | Balance |
| III | 4.6 | 1.2 | 18.7 | 1.19 | Balance |

The most common feature of the examined industry samples was check cracking. All samples contained check cracking in the range of a 5 to 10 millimetre mesh over the entire surface of the hardfacing overlay. The majority of check cracks extended to the substrate-hardface interface. In some instances the check cracks further branched and propagated along the substrate-hardface interface. The propagation of these interface cracks could lead to sections of the overlay being removed from the surface.

The microstructure of the overlay gives rise to its wear properties and so is important for optimising wear performance. The overlay microstructure in the examined samples was a hypereutectic high chromium white iron microstructure consisting of primary M₇C₃ carbide rods in a eutectic composition of austenite and eutectic M₇C₃ carbides. However, the microstructures examined also consisted of undesirable features such as complex regular and interconnected carbides.

Figure 9 shows a desirable microstructure for as deposited hardfacing. Figure 9 is from Sample II in Table V, but is not representative of that sample or any other sample. The microstructure of Figure 9 has been etched in acid ferric chloride. The microstructure consists of hexagonal rods of primary M₇C₃ carbide (white) in a eutectic matrix of M₇C₃carbide and austenite. The primary carbide rods are almost perpendicular to the plane in which Figure 9 was taken and hence appear almost hexagonal, while cellular austenite halos are evident around the primary carbides. The appearance of the carbide rods will vary depending on their orientation, so rather than appearing as hexagons, the primary carbides have a long rod like shape in sections extending perpendicular to the plane in which the photomicrograph of Figure 9 was taken.

When there is sufficient undercooling of the melt, i.e. cooling of the liquid below its normal solidification temperature, before solidification actually occurs, then the normal eutectic as seen in Figure 9 is not produced, but rather an interconnected branched array of finer carbide rods in austenite as shown in Figure 10, taken from Sample III of Table V. The microstructure of Figure 10 is representative of all samples, including Sample II from which the non-representative microstructure of Figure 9 was taken.

In Figure 10, for which acid ferric chloride etchant again was used, the eutectic is still made up of a mixture of M₇C₃ carbide rods (white) and austenite, with the orientation of the carbide rods being roughly planar to the section on which Figure 10 was taken. This undercooled eutectic is referred to as a complex regular eutectic. The eutectic rods are about one fifth the diameter of the primary carbide rods shown in Figure 9 and have a three-fold rotational symmetry which gives rise to the triangular appearance of the carbide clusters. Due to the interconnectivity of the rods this microstructure provides long interconnected paths for crack propagation. The microstructure of Figure 10 therefore is highly undesirable, although it is usual in weld deposited high chromium white irons prior to the present invention.

We have previously shown by electron backscatter diffraction (EBSD) and X-ray diffraction of deep etched samples that the carbide rods in all of these equilateral triangles of complex regular eutectic are interconnected. The carbide rods in the complex regular are M₇C₃ and have the same hexagonal cross section as the primary M₇C₃ carbides, although the complex regular carbides are finer, by approximately 5 times, than the primary carbides. It is not uncommon for "grains" of complex regular structure to be measured in millimetres. Cracking through this complex regular microstructure is shown in more detail in Figures 11(a) and 11(b) for sample II.

The more desirable eutectic microstructure is shown in Figure 9, also for Sample II, because there is considerably reduced interconnectivity of the rods in the eutectic. The microstructure comprises rods of primary M₇C₃ in a matrix of eutectic M₇C₃ and austenite, and a substantial absence of the complex regular microstructure with its attendant interconnected carbide.

There are other high chromium white iron microstructures where the carbides are interconnected and contribute to the embrittlement of hypereutectic high chromium white iron weld deposits. These are when branched primary M₇C₃ carbides are present, as in Figure 12 for Sample III, or a mixture of branched primary M₇C₃ and the complex regular structure is present, as in Figure 13 also from Sample III. Increasing the silicon content of the alloy or increasing the cooling rate tends to promote these two structures.

As mentioned, the branched primary carbides and the complex regular microstructure are favoured by high silicon contents, and the faster cooling rates inherent in weld deposition, which result in undercooling. The growth of these carbides is not determined by the thermal gradient but by the degree of undercooling. Undercooling occurs more readily adjacent to the substrate and hence these carbides can grow in a direction parallel to the substrate rather than perpendicular to the substrate, which is what would be expected if the growth was controlled by the thermal gradient.

This provides one explanation for the check cracking seen in the hardfacing of the industry samples. As shown in Figure 7, the check cracking appears as a square mesh at the surface of the overlay although they have been initiated close to the surface of the substrate. Those appearing at the surface of the overlay have therefore propagated all the way from the substrate to the overlay surface. This cracking pattern is a result of the effect of residual stress due to solidification of the weld bead and the alignment of the carbide rods. Away from the substrate the carbides are likely to grow parallel to the thermal gradient, that is at right angles to the substrate.

A further explanation is provided by close examination of the electron micrograph of Figure 14. Sample III was the source for Figure 14, although it is typical of the high magnification secondary electron images taken of the high chromium weld overlays of each of Samples I, II and III. Although Figure 14 is an image of eutectic carbide and austenite the same discussion can be applied to primary carbides in an austenite matrix.

It has been well established that the preferred crack path in high chromium white iron overlays is along the interface between the carbide and the austenite. The thin dark region (less than 0.2µm thick in the image of Figure 14) surrounding the carbide particles is a thin layer of martensite. Martensite needles can also be seen to extend from these thin layers into the austenite. The brittle martensite surrounding the carbide particles provides an ideal path for crack propagation under conditions of residual stress. In the absence of this martensitic layer, the tougher austenite would be able to absorb the residual stresses and cracking at the interfaces between M₇C₃ carbide and austenite should not occur.

It can be concluded that the presence of branched primary carbide or complex regular, both of which have interconnected carbides, or the presence of martensite at the carbide austenite interface will promote cracking. If these constituents can be eliminated check cracking of the weld deposits should also be eliminated.

Two hypoeutectic, high chromium white irons have been weld deposited on a mild steel disc using plasma transferred arc (PTA). The powder compositions are set out in Table VI.

**Table VI**

| Depositions According to the Invention | | | | | | | |
|---|---|---|---|---|---|---|---|
| | C | Mn | Si | Cr | Ni | Mo | Fe/Impurities |
| Alloy 1 | 2.35 | 3:21 | 0.5 | 20.58 | 3.34 | 0.04 | Balance |
| Alloy 2 | 2.25 | 2.86 | 0.47 | 19.51 | 2.97 | 0.04 | Balance |

The weld depositions were found to be of excellent quality. Figure 15 is a photomacrograph of a two layer weld deposited section which is typical of the deposits for each of the sections. As can be seen, the deposit has a smooth, glossy surface which is substantially free of slag and which does not exhibit any surface cracks. Also, presentation of a magnet to the weld deposit does not exhibit any ferromagnetic attraction indicative of the presence of martensite.

The above description in relation to Samples I, II and III, illustrated with reference to Figures 7 to 14, focuses principally on the adverse consequences of interconnectivity of M₇C₃ primary carbides. However, as indicated in relation to Figure 14, those samples exhibited detectable martensite at M₇C₃ carbide and austenite interfaces, such that each of Samples I, II and III exhibited strong ferromagnetism able to be attributed only to the presence of the martensite. That is, the weld deposits of Samples I, II and III strongly attracted a magnet when presented to each of those deposits.

Figures 16 and 17 are photomicrographs respectively taken longitudinally and transversely with respect to a weld bead of the deposit.

As is evident from Figures 15, 16 and 17, the weld deposit were substantially crack free. The microstructure is characterised by dendrites and a eutectic of M₇C₃ and austenite and an absence of martensite at M₇C₃ carbide and austenite interfaces. Also, the M₇C₃ carbide shows a low level of interconnectivity. Both powders resulted in excellent fluidity, while the level of dilution was good in being approximately 10 to 25%. The substrate preheat level required was much lower than used in current practice, at 150°C rather than about 300°C.

Finally, it will be appreciated that there may be other modifications and changes made to the embodiments described above that may also be within the scope of the present invention.

## Claims

1. A method of producing a wear resistant, high chromium white iron casting, the method comprising:
- casting a melt of a high chromium white cast iron, wherein said melt contains at least one martensite promoter selected from the group of silicon at a level from 0.25 to 3.5% and boron at a level of up to 2%, and at least one austenite stabiliser, selected from the group of manganese, nickel, copper and molybdenum at a level of from 4 to 12% for each of manganese, nickel, and copper, and an effective equivalent of molybdenum after allowance for a proportion of molybdenum taken up as carbide,
- cooling the melt so as to produce a casting having a microstructure which in an unheat-treated condition includes austenite and M₇C₃ carbides,
**characterized in that**
the level of the martensite promoter in the melt, the level of the austenite stabiliser in the melt and the cooling rate are selected so as to achieve a balance between the effects of these variables and to thus obtain a white iron casting which in an unheat-treated condition has a microstructure that is free of martensite at interfaces between the austenite and M₇C₃ carbides.

2. The method of claim 1, wherein the martensite promoter silicon is present at a level of from 0.5 to 3.25%.

3. The method of claim 1, wherein the martensite promoter boron is present at a level of up to 1%.

4. The method of any one of claims 1 to 3, wherein the austenite stabiliser is present at a level of from 4 to 8% for each of manganese, nickel, and copper and an effective equivalent of molybdenum after allowance for a proportion of molybdenum taken up as carbide.

5. The method of any one of claims 1 to 4, wherein the level of the martensite promoter in the melt or the high chromium white cast iron material, the level of the austenite stabiliser in the melt or the high chromium white cast iron material and the cooling rate are selected so as to achieve a balance between the effects of these variables and to thus obtain a white iron casting or a hardfacing on the substrate which in an unheat-treated condition has a microstructure wherein the M₇C₃ carbides exhibit a level of interconnectivity which results in the microstructure being substantially free of branched carbide particles.

6. The method of any one of claims 1 to 5, wherein the high chromium white cast iron or the high chromium white cast iron material is of a hypoeutectic composition, and said interfaces include interfaces between primary austenite and eutectic M₇C₃ carbide and between eutectic austenite and eutectic M₇C₃ carbide.

7. The method of any one of claims 1 to 5, wherein the high chromium white cast iron or the high chromium white cast iron material is of a eutectic composition, with said interfaces being between eutectic austenite and eutectic M₇C₃ carbide.

8. The method of any one of claims 1 to 5, wherein the high chromium white cast iron or the high chromium white cast iron material is of a hypereutectic composition, and said interfaces include interfaces between primary M₇C₃ carbide and eutectic austenite and between eutectic austenite and eutectic M₇C₃ carbide.

9. The method of claim 6, wherein the high chromium white cast iron or the high chromium white cast iron material has from 1.0 to 3.0% C, 18.0 to 27.0% Cr, 4.0 to 8.0% Ni, 0.25 to 2.75% Si, and optionally 4.0 to 8.0% Mn, and a balance, apart from other incidental alloy elements and impurities, of Fe.

10. The method of claim 6, wherein the high chromium white cast iron or the high chromium white cast iron material has 2.5 to 4.0% C, 18.0 to 27.0% Cr, 4.0 to 8.0% Ni, 0.25 to 2.75% Si, up to 10% each of at least one of Nb and V, and optionally 4.0 to 8.0% Mn, and a balance, apart from other incidental alloying elements and impurities, of Fe.

11. The method of claim 7, wherein the high chromium white cast iron or the high chromium white cast iron material has from 3.0 to 4.0% C, 15.0 to 27.0% Cr, 4.0 to 8.0% Ni, 0.25 to 2.75% Si, and optionally 4.0 to 8.0% Mn, and a balance, apart from other incidental alloy elements and impurities, of Fe.

12. The method of claim 7, wherein the high chromium white cast iron or the high chromium white cast iron material has 4.25 to 4.75% C, 15.0 to 27.0% Cr, 4.0 to 8.0% Ni, 0.25 to 2.75% Si, up to 10% each of at least one of Nb and V, and optionally 4.0 to 8.0% Mn, and a balance, apart from other incidental alloying elements and impurities, of Fe.

13. The method of claim 8, wherein the high chromium white cast iron or the high chromium white cast iron material ron has from 4.0 to 5.0% C, 20.0 to 27.0% Cr, 4.0 to 8.0% Ni, 0.25 to 2.75% Si, and optionally 4.0 to 8.0% Mn, and a balance, apart from other incidental alloy elements and impurities, of Fe.

14. The method of claim 8, wherein the high chromium white cast iron or the high chromium white cast iron material iron has 5.0 to 6.0% C, 20.0 to 27.0% Cr, 4.0 to 8.0% Ni, 0.25 to 2.75% Si, up to 10% each of at least one of Nb and V, and optionally 4.0 to 8.0% Mn, and a balance, apart from other incidental alloying elements and impurities, of Fe.

15. The method of any one of claims 1 to 14, wherein at least two austenite stabilisers are present, and the combined level of austenite stabiliser is not in excess of 20%.

16. The method of any one of claims 1 to 14, wherein at least two austenite stabilisers are present, and the combined level of austenite stabiliser is not in excess of 16%.
